

- [54] **ELECTRICALLY-CONDUCTIVE CERAMIC-METALLIC PROTECTIVE COATING**
- [75] Inventor: **Harold J. Michael**, Columbus, Ohio
- [73] Assignee: **Rockwell International Corporation**, Pittsburgh, Pa.
- [22] Filed: **Mar. 6, 1972**
- [21] Appl. No.: **232,302**

**Related U.S. Application Data**

- [62] Division of Ser. No. 93,493, Nov. 27, 1970, Pat. No. 3,702,770.
- [52] **U.S. Cl. ... 117/105.2, 117/93.1 PF, 117/169 R, 117/129**
- [51] **Int. Cl. .... B44d 1/08**
- [58] **Field of Search**..... 106/39 R, 313; 29/182.5, 29/195; 75/94; 148/26; 219/146; 117/105.2, 46 FS, 22, 129, 93.1 PF

**[56] References Cited****UNITED STATES PATENTS**

- |           |         |                        |         |
|-----------|---------|------------------------|---------|
| 2,697,159 | 12/1954 | Donahey.....           | 106/313 |
| 2,745,769 | 5/1956  | Linnert et al. ....    | 117/129 |
| 2,775,531 | 12/1956 | Montgomery et al. .... | 117/22  |

|           |         |                      |           |
|-----------|---------|----------------------|-----------|
| 2,848,349 | 8/1958  | Rechter et al. ....  | 117/105.2 |
| 2,904,449 | 9/1959  | Bradstreet.....      | 117/105.2 |
| 3,322,515 | 5/1967  | Dittrica et al. .... | 29/191.2  |
| 3,388,001 | 6/1968  | Blum et al. ....     | 117/105.2 |
| 3,397,080 | 8/1968  | Girard et al. ....   | 117/105.2 |
| 3,607,343 | 9/1971  | Longo et al. ....    | 117/105.2 |
| 3,702,770 | 11/1972 | Michael .....        | 117/105.2 |
| 3,706,579 | 12/1972 | Michael .....        | 106/1     |

**FOREIGN PATENTS OR APPLICATIONS**

- |           |        |               |         |
|-----------|--------|---------------|---------|
| 1,080,383 | 4/1960 | Germany ..... | 219/146 |
|-----------|--------|---------------|---------|

**OTHER PUBLICATIONS**

E. Levin et al., Phase Diagrams for Ceramists, Columbus, 1964, p. 172 (LiAO-SiO<sub>2</sub>-TiO<sub>2</sub>).

*Primary Examiner*—Michael Sofocleous

**[57] ABSTRACT**

Compositions having essentially only ceramic and metallic constituents are provided for application to metal parts by conventional oxyacetylene flame spraying equipment or plasma arc spraying equipment to develop an adhering electrically-conductive protective coating to thereby provide improved metal part resistance to surface corrosion attack.

**6 Claims, No Drawings**

# ELECTRICALLY-CONDUCTIVE CERAMIC-METALLIC PROTECTIVE COATING

## CROSS-REFERENCE

This is a division, of application Ser. No. 93,493, filed Nov. 27, 1970, now U.S. Pat. No. 3,702,770.

## SUMMARY OF THE INVENTION

Aluminum metal powder is mixed in prescribed proportions with a finely divided alkali titanate compound, such as lithium-silico-titanate (lithium titanium silicate), lithium titanate, or both, by way of example, for subsequent application to any of a number of different metal parts using conventional oxyacetylene flame spray equipment or plasma arc equipment to thereby develop improved metal part resistance to surface corrosion. The specified compositions are suitable for application in the same manner over metal part weld areas, including application over weld areas that join metal parts previously coated with different but compatible types of fused-on ceramic-metallic protective coatings.

## DETAILED DESCRIPTION

The following general formulation identifies the principal constituents, by range and on a 100 parts by weight basis, of the ceramic-metallic protective coating compositions of this invention:

### COATING COMPOSITIONS

| Constituent                                                 | Range   |
|-------------------------------------------------------------|---------|
| Aluminum metal powder, -120 +325 mesh, spherical particles, | 20 - 80 |
| Alkali titanate compound, -120 +325 mesh frit,              | 20 - 80 |
| TOTAL.                                                      | 100.0   |

Details regarding each of the principal constituents, and particularly methods for formulating and preparing certain of such principal constituents, are provided in those portions of the detailed description which follow.

Adjustments may be made to the composition formulation within the ranges indicated to vary the degree of resistance to weathering and corrosion attack obtained for particular metal parts coated with the instant composition and also to vary the ease of application obtained with conventional spraying equipment of the oxyacetylene type or plasma arc type as a function of the composition wetting property.

### ALUMINUM POWDER CONSTITUENT

The ceramic-metallic composition of this invention utilizes -120 mesh +325 mesh aluminum powder such as is commonly purchased commercially in a spray grade form, such metal powder having particles which are substantially spherical in configuration.

### ALKALI TITANATE COMPOUND CONSTITUENT

One preferred alkali titanate compound constituent is lithium-silico-titanate, sometimes referred to herein as lithium titanium silicate, an essentially non-homogeneous opalescent glass having two distinct compositional phases in both the liquid condition and the solid condition. Such constituent is preferably com-

pounded to have a 1:1:1 molecular ratio of  $\text{Li}_2\text{O}$  to  $\text{SiO}_2$  to  $\text{TiO}_2$  and may be made in the following manner.

The Example I ingredients given below, stated on a 100 parts total weight basis, are combined by thorough dry blending, smelted at 2,000° F. - 2,300° F., and fritted to form the preferred lithium-silico-titanate compound constituent:

### EXAMPLE I - CONSTITUENT COMPOSITION

| Component                                      | Range       | Preferred Amount |
|------------------------------------------------|-------------|------------------|
| Silica ( $\text{SiO}_2$ )                      | 20.0 - 80.0 | 28.2             |
| Titania ( $\text{TiO}_2$ )                     | 20.0 - 80.0 | 37.3             |
| Lithium Carbonate ( $\text{Li}_2\text{CO}_3$ ) | 12.4 - 74.0 | 34.5             |
| TOTAL                                          | 100.0       | 100.0            |

The resulting frit has two compositional phases in both the liquid condition and the solid condition and is graded for use to pass a No. 120 U.S. standard sieve but remain on a No. 325 U.S. standard sieve. Particles larger than 120 mesh may be further ground for use; particles of a -325 mesh size may be re-charged into subsequent constituent batches as cullet for re-firing.

From a calculated oxide content standpoint the above detailed lithium-silico-titanate compound constituent used in the instant invention has the following composition on a 100 parts by weight basis after smelting:

| Oxide                 | Range   | Preferred Amount |
|-----------------------|---------|------------------|
| $\text{Li}_2\text{O}$ | 5 - 30  | 17.6             |
| $\text{TiO}_2$        | 20 - 80 | 47.0             |
| $\text{SiO}_2$        | 20 - 80 | 35.4             |
| TOTAL                 | 100.0   | 100.0            |

Another alkali titanate compound constituent satisfactory for practice of this invention is lithium titanate. Such may be included in the compositions of this invention optionally or additionally with respect to lithium-silico-titanate, for example. If provided by way of addition, the compound functions to further decrease the electrical surface resistivity property of the final coating to thereby develop improved anodic protection for the resulting coated metal part. The below detailed lithium titanate constituent, however, does not in most cases alone provide optimum surface wetting during application of the composition to metal parts by flame spraying. Such lithium titanate constituent is compounded to have a preferred 1:1 molecular ratio of  $\text{TiO}_2$  to  $\text{LiO}_2$  and may be made from the following Example II ingredients, detailed on a 100 parts total weight basis:

### EXAMPLE II - CONSTITUENT COMPOSITION

| Component                                      | Preferred Amount |
|------------------------------------------------|------------------|
| Lithium Carbonate ( $\text{Li}_2\text{CO}_3$ ) | 48.1             |
| Titania ( $\text{TiO}_2$ )                     | 51.9             |
| TOTAL                                          | 100.0            |

The ingredients of the constituent are combined by thorough blending (either wet or dry) and fused into clinker form in an air furnace at a temperature of approximately 2,000° F. ± 50° F. for subsequent crushing and screening. The above Example II ingredients may

alternatively be melted at a temperature of approximately 2,300° F.  $\pm$  50° F. and fritted in lieu of being fused into clinker form for the subsequent processing.

The resulting ground clinker or frit is graded to pass a No. 120 U.S. standard sieve and remain on a No. 325 U.S. standard sieve for use. As in the case of the lithium titanium silicate constituent, particles larger than 120 mesh may be further ground for use; particles of a -325 mesh size may be re-charged into subsequent lithium titanate constituent batches as cullet for refiring.

It should be noted that other alkali titanates may be used in the coating composition formulations although lithium titanate compounds are preferred inasmuch as lithium is more electro-positive and provides superior anodic protection in comparison to other alkali metal titanates such as sodium titanate or potassium titanate or in comparison to alkali earth metal titanates such as the titanates of magnesium, calcium, strontium, or barium. Stated in another manner, lithium titanate compounds appear to particularly enhance or improve the electrical surface conductivity of the applied coating.

The following Example III, Example IV, and Example V coating composition formulations, given on a 100 parts by total weight basis, are examples of embodiments of this invention that have been utilized for satisfactorily developing improved resistance to corrosion attack for metal parts to which the composition has been applied.

#### EXAMPLE III - COATING COMPOSITION

| Constituent                                                          | Preferred Amount |
|----------------------------------------------------------------------|------------------|
| Aluminum metal powder, -120 +325 mesh spherical particles,           | 40               |
| Lithium-silico-titanate, -120 +325 mesh frit,                        | 40               |
| Lithium titanate ( $\text{Li}_2\text{TiO}_3$ ), -120 +325 mesh frit, | 20               |
| <b>TOTAL</b>                                                         | <b>100</b>       |

#### EXAMPLE IV - COATING COMPOSITION

| Constituent                                                | Preferred Amount |
|------------------------------------------------------------|------------------|
| Aluminum metal powder, -120 +325 mesh spherical particles, | 50               |
| Lithium-silico-titanate, -120 +325 mesh frit,              | 50               |
| <b>TOTAL</b>                                               | <b>100</b>       |

#### EXAMPLE V - COATING COMPOSITION

| Constituent                                                          | Preferred Amount |
|----------------------------------------------------------------------|------------------|
| Aluminum metal powder, -120 +325 mesh spherical particles,           | 50               |
| Lithium titanate ( $\text{Li}_2\text{TiO}_3$ ), -120 +325 mesh frit, | 50               |
| <b>TOTAL</b>                                                         | <b>100</b>       |

Details with respect to application of any of the above Example III through V coating compositions to metal parts by flame spraying are given below.

The desired constituents of -120 +325 mesh screen size for a particular coating composition prior to application of the composition to a metal part by flame spraying are first carefully weighed to the proper proportions and then dry blended until a uniform color is obtained. Flame spraying, as suggested previously, is then accomplished using either conventional oxyacetylene flame spray equipment or conventional plasma arc flame spraying equipment depending upon availability.

In either case, however, it is necessary that the metal part, which may be a large mild steel structural part by way of example, should be cleaned by mechanical means in those areas which are to be coated. Cleaning may be accomplished either by abrasive blasting using a 40 - 80 mesh clean sand or alundum grit, by disc sanding, or by stiff wire brushing. The areas to be coated basically must be free of oxide, scale, welding flux, and other foreign material prior to application of the coating composition. Since roughened, clean metal surface is essential to good adherence, any loose particles should therefore be removed from the metal part surface as by blowing using clean, dry, compressed air.

- 15 Using conventional oxyacetylene flame spray equipment, by way of example a Metco powder spray gun with a ceramic material feed nozzle having a No. 2 feed orifice, the compositions are applied by box or cross coating the metal part practicing the following steps.
- 20 First, and prior to starting the flow of composition through the gun, pre-heat the surface to be initially sprayed by passing the gun flame over the surface at a distance of from 6 inches to 8 inches thereby accomplishing a degree of pre-heating. Next, composition flow is started, adopting the equipment manufacturer's control setting recommendations as to feed setting, oxygen flow, and acetylene flow, and application is accomplished by spraying the metal part surface using horizontal straight-line rather than arc-type motion
- 25 with the composition material impinging upon the metal part surface at as near a 90° angle as possible. After the pre-heating has been accomplished with respect to the area to be initially coated, the remainder of the metal part is normally automatically pre-heated as the spraying work progresses. Adequate coverage of the metal part is usually obtained using one cross or box coat with a composition deposit density of from 20 to 23 grams of composition per square foot of metal part surface. Care must be taken that the speed of application is not so fast as to produce a loose, powdery-type coating. Normally non-porous coating is obtained with gun travel over the work at a velocity of not more than four feet per minute.

The non-porous composition coating as sprayed has excellent bond in adhesion as well as cohesion. The coating composition as sprayed provides excellent long time anodic protection for numerous different ferrous metals, stainless steels, and nickel-base alloys exposed to salt corrosion environments. In some cases (Example I, Example III formulations) the applied intermetallic compound coating has essentially a zero resistance to electrical current flow with as little as 40 percent to 50 percent by weight aluminum metal content. In addition, the coating has outstanding resistance to impact, bending, or deformation failure by virtue of a high degree of inherent ductility. The coating is compatible with fused-on type of cermet protective coatings, such as the coatings detailed in my co-pending Application for U.S. Letters Patent Ser. No. 69,914 filed Sept. 4, 1970 (a continuation-in-part of Application for United States Letters Patent Ser. No. 833,698, filed June 16, 1969 and assigned to the assignee of this application), now U.S. Letters Pat. No. 3,706,579 granted Dec. 19, 1972, and has also been successfully applied over conventional welds that serve to join two metal parts previously coated with such fused-on type of cermet protective coatings.

I claim:

1. The method of providing a metal surface with an adhered, highly-conductive protective coating comprising the steps of:

- a. Combining, on a 100 parts total weight basis, from 20 to 80 parts aluminum metal in finely divided sprayable powder form with from 20 to 80 parts alkali titanate from the group consisting of lithium titanate, lithium-silico-titanate, and mixtures of lithium titanate and lithium-silico-titanate in finely divided frit form,
- b. Thoroughly mixing said aluminum metal powder and said alkali titanate frit to form a particulate coating mixture of uniform consistency,
- c. Flowing said uniform particulate coating mixture in a temperature-elevated gaseous stream, and
- d. Projecting said temperature-elevated gaseous stream containing said uniform particulate coating mixture toward said metal surface at a rate and with sufficient force to thereby impinge and adhere said particulate coating mixture on said metal surface at a substantially elevated temperature, said particulate coating mixture impinged on said metal surface at an elevated temperature forming on said metal surface an aluminum metal and alkali tita-

25

nate protective coating having a surface electrical resistivity of substantially zero.

2. The method defined by claim 1 wherein said uniform particulate coating mixture composition consists of approximately 40 parts by weight of aluminum metal powder, 40 parts by weight of lithium-silico-titanate, and 20 parts by weight of lithium titanate.

3. The method defined by claim 1 wherein said uniform particulate coating mixture composition consists of approximately 50 parts by weight of aluminum metal powder and 50 parts by weight of lithium titanate.

4. The method defined by claim 1 wherein said uniform particulate coating mixture composition consists of approximately 50 parts by weight of aluminum metal powder and 50 parts by weight of lithium-silico-titanate.

5. The method defined by claim 2 wherein said lithium-silico-titanate on a calculated oxide content basis consists of lithium oxide, silicon oxide, and titanium oxide in an approximately 1:1:1 molecular ratio.

6. The method defined by claim 4 wherein said lithium-silico-titanate on a calculated oxide content basis consists of lithium oxide, silicon oxide, and titanium oxide in an approximately 1:1:1 molecular ratio.

\* \* \* \* \*

30

35

40

45

50

55

60

65